

Patented Apr. 6, 1926.

1,579,801

# UNITED STATES PATENT OFFICE.

JOSEPH E. BABB, OF PITTSBURGH, PENNSYLVANIA, ASSIGNOR TO WAVERLY OIL WORKS COMPANY, OF PITTSBURGH, PENNSYLVANIA, A CORPORATION OF PENNSYLVANIA.

## EXPLOSIVE FUEL MIXTURE AND METHOD OF MAKING THE SAME.

No Drawing.

Application filed December 15, 1924. Serial No. 756,071.

To all whom it may concern:

Be it known that I, JOSEPH E. BABB, a citizen of the United States, and a resident of Pittsburgh, in the county of Allegheny and 5 State of Pennsylvania, have invented a new and useful Improvement in Explosive Fuel Mixtures and Methods of Making the Same; and I do hereby declare the following to be a full, clear, and exact description thereof.

10 My invention relates to a fuel mixture for use in internal combustion engines, for the purpose of permitting increase of compression and effecting more uniform compression in the engine cylinders.

15 One object of my invention is to provide a lead compound that is soluble in gasoline, kerosene and other motor fuels, to increase the effectiveness thereof, but which is nevertheless not dangerous to the life and health 20 of those engaged in its manufacture.

Another object of my invention is to provide a mixture containing lead soap that is soluble in gasoline and benzol, which does not belong to the alkyl and phenyl com- 25 pounds, nor to the ethyl or methyl groups of hydrocarbons, of the type formulas  $C_nH_{2n+2}$  and  $C_nH_{2n}$ , for example.

Another object of my invention is to provide an improved mixture and method of 30 making the same that is of simple composition, effective in use, and which is not dangerous to the operator either during the stages of manufacture thereof, or when ready for use.

35 I have found that by mixing distilled rosin or distillation products of rosin with an oxide of lead, in the manner hereinafter described, a lead soap is formed that is soluble in gasoline, to the extent of 10%, and 40 is soluble in benzol to the extent of 50%, by weight. When this solution is mixed with gasoline in such quantity that the lead content thereof is one-thousandth part of the whole, a very satisfactory motor fuel is secured, which will permit of materially increased compression without producing "knocks".

In practicing my invention, I first subject the rosin to distillation, preferably in a fire still. The resultant distillate is popularly known as rosin oil. Rosin oil is a commercial commodity and I may prefer to purchase it in the open market.

In the manufacture of my lead compound,

the distilled rosin is heated in an open fire 55 kettle to a temperature of perhaps 140° C., and oxide of lead, such as the monoxide of lead known as litharge, is added to the rosin in quantities sufficient to neutralize the acids of the rosin. The heat is maintained 60 and the mixture is agitated until the oxide of lead has been completely combined with the acids of the rosin.

The foregoing forms what I term a lead soap and is soluble in gasoline and benzol, 65 to the extent of 10% and 50%, respectively, or the solution may be of any strength below saturation. The soap is also soluble in acetone which may be employed instead of gasoline or benzol. This concentrated solution 70 may then be added to the main body of the motor fuel, preferably in such amount that the portion of lead in the fuel is 1 to 1000.

Lead soap may be manufactured also by 75 first neutralizing the rosin acids with an alkali such as caustic soda or potash, to form a soluble soap and then adding a soluble lead salt, such as lead chloride or lead acetate, to change soluble soap to insoluble lead 80 soap. The lead soap is subsequently washed to free it from the soluble alkali salts and then dried. Thereafter it may be mixed with gasoline or benzol, as in the case of the lead soap made after the method above 85 described.

Furthermore, in place of the distilled rosin above described I may employ products obtainable by distillation of crude gums such as fossil gums similar to kauri gum, manila copal, or varnish gums, from which rosin and turpentine are obtained, or from those gums of the conifer species which may be employed in forming soluble lead soaps either through direct combination with the 95 lead or by the distillation process.

I may also employ the resinous element to increase the solubility of metallic soaps other than lead, to thereby render them soluble in benzol, gasoline, acetone, and liquid fuels. 100

It will be apparent that I do not limit myself to the precise steps and proportions set forth in the foregoing specification, but my invention is limited in scope only to the extent defined in the accompanying claims. 105

I claim as my invention:

1. A fuel composition comprising an explosion motor fuel and a gum of resinous

character that is soluble in gasoline, combined with a lead oxide.

2. A motor fuel containing a soap soluble in gasoline, said soap being composed of 5 distillation products of rosin and a lead oxide.

3. The process which comprises heating a distillation product of rosin, adding thereto a lead oxide in sufficient quantity to substantially neutralize the acids of the rosin, 10 dissolving the resultant product in a liquid solvent, and adding the mixture to a motor fuel.

4. The process which comprises heating a 15 distillation product of rosin, adding thereto

a lead oxide in quantity sufficient to substantially neutralize the acids of the rosin, and adding said mixture to a motor fuel.

5. The process which comprises heating a distillation product of rosin, adding thereto 20 a lead oxide, and adding said mixture to a motor fuel.

6. The method of making a fuel mixture which comprises providing a distillation product of resinous gum, combining it with 25 an oxide of lead, and adding the mixture to an explosion motor fuel.

In testimony whereof, I, the said JOSEPH E. BABB, have hereunto set my hand.

JOSEPH E. BABB.